

# United States Patent [19]

Boyko et al.

[11] 3,762,913

[45] Oct. 2, 1973

[54] **ALLOY AND METHOD OF WELDING  
STRUCTURES INCLUDING THIS ALLOY**

[75] Inventors: **Eugene S. Boyko, Monroeville; Clark  
M. Owens, Irwin, both of Pa.**

[73] Assignee: **Westinghouse Electric Corporation,  
Pittsburgh, Pa.**

[22] Filed: **Jan. 17, 1967**

[21] Appl. No.: **611,533**

[52] U.S. Cl. .... **75/122, 75/124, 75/128**

[51] Int. Cl. .... **C22c 39/02, C22c 39/20**

[58] **Field of Search** .... **75/122, 128, 134,  
75/170, 171, 124**

[56] **References Cited**

UNITED STATES PATENTS

|           |         |                 |          |
|-----------|---------|-----------------|----------|
| 2,054,405 | 9/1936  | Becket et al.   | 75/128   |
| 2,054,770 | 9/1936  | Kautz           | 75/128   |
| 2,240,672 | 5/1941  | Scherer et al.  | 75/128 X |
| 3,159,479 | 12/1964 | Copson et al.   | 75/128   |
| 3,177,577 | 4/1965  | Fujimura et al. | 75/128 X |

FOREIGN PATENTS OR APPLICATIONS

114,424 9/1947 Australia ..... 75/171

OTHER PUBLICATIONS

"Properties of Some Metals and Alloys," The International Nickel Co., Inc., New York, page 21, 1962.

*Primary Examiner*—Charles N. Lovell

*Attorney*—A. T. Stratton and Z. L. Dermer

[57]

**ABSTRACT**

An iron-nickel-chromium alloy with which crack-free sound welds are produced for fuel elements and tube-to-tube sheet assemblies having low carbon (0.05 max) and up to 0.40 each of titanium and aluminum, the Ti being eight to 10 times the carbon and the aluminum four to six times the carbon. The Ti and/or Al suppress the formation of massive  $\text{Cr}_{23}\text{C}_6$  molecules.

Also a method of welding iron-nickel-chromium alloy in which Ti and/or Al are present to prevent cracks from forming.

**1 Claim, 28 Drawing Figures**

PATENTED OCT 2 1973

3,762,913

SHEET 01 OF 13



FIG.3.



FIG.2.

WITNESSES

Theodore F. Krolek  
James F. Young

INVENTORS  
Eugene S. Boyko  
and Clark M. Owens  
BY *Jozefina A. Fermer*  
ATTORNEY

PATENTED OCT 21 1973

3,762,913

SHEET 02 OF 13



FIG.4.



FIG.5.

Ti(C,N) PRECIPITATES IN ANNEALED INCOLOY 800

INVENTORS  
Eugene S. Boyko  
and Clark M. Owens  
BY *J. M. Pearson*  
ATTORNEY

PATENTED OCT 2 1973

3,762,913

SHEET 03 OF 13



FIG. 6.

TiC, TiN, Cr<sub>23</sub>C<sub>6</sub> PRECIPITATES IN ANNEALED INCOLOY 800



FIG. 7.

Cr<sub>23</sub>C<sub>6</sub> PRECIPITATES IN ANNEALED INCOLOY 800

INVENTORS

Eugene S. Boyko  
and Clark M. Owens

BY *Jernimold S. Jerome*  
ATTORNEY

PATENTED OCT 2 1973

3,762,913

SHEET 04 OF 13



FIG. 8

$\text{Cr}_{23}\text{C}_6$  DENDRITE IN ANNEALED INCOLOY 800



FIG. 9.

ELECTRON DIFFRACTION PATTERN OF A DENTRITIC  
PRECIPITATE IDENTIFIED AS  $\text{Cr}_{23}\text{C}_6$

INVENTORS

Eugene S. Boyko  
and Clark M. Owens

BY *J. Berner*  
ATTORNEY

PATENTED OCT 2 1973

3,762,913

SHEET 05 OF 13

CRACK



FIG.10.

WELD PUDDLE CRACKING IN ANNEALED INCOLOY 800



FIG.10A.

$\text{Cr}_{23}\text{C}_6$  DENDRITE IN AN EARLY STAGE OF DEVELOPMENT  
EXTRACT FROM WELD OF ANNEALED INCOLOY 800

INVENTORS

Eugene S. Boyko  
and Clark M. Owens

BY *J. S. Fermer*  
ATTORNEY

PATENTED OCT 2 1973

3,762,913

SHEET 06 OF 13



FIG.II.

TYPICAL ELECTRON MICROSTRUCTURE OF  $\frac{1}{4}$ " INCOLOY 800 PLATE  
SHOWING GRAIN BOUNDARY PRECIPITATES



FIG.I2.

Ti(C,N)  
BAR STOCK -  $\frac{5}{8}$ " DIAMETER B-O ALLOY  
NOTE LARGE Ti(C,N) CARBIDES

INVENTORS

Eugene S. Boyko  
and Clark M. Owens  
BY *Jegmund L. Turner*  
ATTORNEY

PATENTED OCT 2 1973

3,762,913

SHEET 07 OF 13



FIG.13.

TYPICAL ELECTRON MICROSTRUCTURE OF  $5\frac{1}{8}$ " DIAMETER  
B-O ALLOY BAR STOCK



FIG.14.

TYPICAL ELECTRON MICROSTRUCTURE OF  $5\frac{1}{8}$ " DIAMETER  
B-O ALLOY BAR STOCK

INVENTORS

Eugene S. Boyko  
and Clark M. Owens

BY *J. Michael S. Fermer*

ATTORNEY

PATENTED OCT 2 1973

3,762,913

SHEET 08 OF 13



FIG.15.

ELECTRON TRANSMISSION OF  $5/8$ " DIAMETER B-O ALLOY BAR STOCK  
NOTE PRESENCE OF DISLOCATIONS ASSOCIATED WITH PRECIPITATES



FIG.16.

ELECTRON MICROSTRUCTURE OF 0.010" WALL



FIG.17.

ELECTRON MICROSTRUCTURE OF 0.010" WALL

INVENTORS

Eugene S. Boyko  
and Clark M. Owens

BY *Jozefina J. Fermer*  
ATTORNEY

PATENTED OCT 2 1973

3,762,913

SHEET 09 OF 13



FIG.18.

SPECIMEN OF -0.010" WALL TUBING



FIG.19.

B-O ALLOY WELDED WITH Ni 82 FILLER WIRE

INVENTORS

Eugene S. Boyko  
and Clark M. Owens

BY *J. J. Givens*  
ATTORNEY

PATENTED OCT 2 1973

3,762,913

SHEET 10 OF 13



FIG.20.

B-0 ALLOY WELDED WITH INCO 138 BARE FILLER WIRE



FIG.21.

B-0 ALLOY WELDED WITH 330 STAINLESS FILLER WIRE

INVENTORS

Eugene S. Boyko  
and Clark M. Owens  
BY *J. Ignatius Lehman*  
ATTORNEY

PATENTED OCT 2 1973

3,762,913

SHEET 11 OF 13



FIG.22.

B-0 ALLOY TO 304 SS WELDED WITH NI 82 FILLER



FIG.23.

B-0 ALLOY TO 304 SS WELDED WITH INCO 138 BARE FILLER WIRE

INVENTORS

Eugene S. Boyko  
and Clark M. Owens  
BY *Zigmund S. Fermer*  
ATTORNEY

PATENTED OCT 2 1973

3,762,913

SHEET 12 OF 13



FIG.24.

B-0 ALLOY TO 304 SS WELDED WITH 330 SS FILLER WIRE



FIG.25.

B-0 ALLOY TO 316 SS WELDED WITH Ni 82 FILLER WIRE

INVENTORS

Eugene S. Boyko  
and Clark M. Owens  
BY *Zigmund L. Ferenc*  
ATTORNEY

PATENTED OCT 2 1973

3,762,913

SHEET 13 OF 13



FIG.26.

B-0 ALLOY TO 316 SS WELDED WITH INCO 138 FILLER WIRE



FIG.27.

B-0 ALLOY TO 316 SS WELDED WITH 330 SS FILLER WIRE

INVENTORS

Eugene S. Boyko  
and Clark M. Owens

BY *Zygmund S. Turner*  
ATTORNEY

**ALLOY AND METHOD OF WELDING  
STRUCTURES INCLUDING THIS ALLOY**

**BACKGROUND OF THE INVENTION**

This invention relates to the ferrous-alloy art and has particularly relationship to the fabrication by welding of structures including parts of iron-nickel-chromium alloys.

An iron-nickel-chromium alloy, sold by International Nickel Company under the name Incoloy 800, and having approximately 45 percent iron, 32 percent nickel and 21 percent chromium has been found to have advantageous properties for use in power-generation apparatus in which the heat-exchange fluid is a corrosive material such as liquid sodium. Typically, this alloy has the following composition:

TABLE I

|              |              |      |      |              |      |
|--------------|--------------|------|------|--------------|------|
| C            | Mn           | Fe   | S    | Si           | Cu   |
| 0.10<br>max. | 1.50<br>max. | Bal. | 0.03 | 1.00<br>max. | max. |
| Ni           | Cr           |      |      |              |      |
| 30-35        | 19-23        |      |      |              |      |

This alloy has favorable high-temperature mechanical properties, particularly high tensile-stress resistance and high ductility at temperatures of 1,150° F., and it also has corrosion resistance at the same high temperatures to liquid sodium and steam. Attempts have been made to use this alloy for cladding for fuel elements and for tube-to-plate or tube-to-tube sheet assemblies of heat exchangers. Such use requires that the cladding or assemblies be sealed by sound pressure-tight welds which must necessarily be crack-free. This requirement is particularly stringent as to assemblies in the light of the 20 or 30 year design life which is demanded of heat exchangers. The attempts have failed because it has not been possible to produce crack-free welds.

It is an object of this invention to overcome the above-described disability of the iron-nickel-chromium alloy and to provide an alloy of the iron-nickel-chromium type with which crack-free welds shall be readily producible and to provide cladding for power generators and tube-to-plate assemblies using this alloy.

It is also an object of this invention to provide a novel method for producing crack-free welds with iron-nickel-chromium alloys.

This invention arises from the discovery that the cracks in the welds are caused by the presence of chromium carbides, particularly massive molecules of  $\text{Cr}_{23}\text{C}_6$  in the parts used and their formation, during the welding operation. These chromium carbides precipitate in grain boundaries in the sheet and tubes used to make the structures and during the welding operation these carbides and others, produced under the heat of the welding arc, cause the cracks to form. In accordance with this invention, the formation of cracks is suppressed by including in the alloy adequate material having an affinity for carbon which may form carbides or nitrides dispersed throughout the matrix. An important such material is titanium; aluminum also serves as such material; and both Ti and Al may be used.

Another aspect of this invention is to maintain the carbon at a low magnitude. Specifically, an iron-nickel-chromium alloy is provided in which the carbon is maintained at less than about 0.05 percent and the tita-

nium is maintained at between eight and 10 times the carbon content. The alloy according to this invention is herein called B-0 Alloy.

A recommended composition in accordance with this invention of this B-0 Alloy, with which are produced crack-free welded structures having high resistance to tensile stress and high ductility at high temperatures of about 1,150° F. and high corrosion resistance to steam and liquid sodium at these high temperatures, is as follows:

TABLE II

|             |              |              |                      |                     |             |
|-------------|--------------|--------------|----------------------|---------------------|-------------|
| C           | Mn           | S            | P                    | Si                  | Ni          |
| .05<br>max. | 1.50<br>max. | .030<br>max. | .03<br>max.          | 1.0<br>max.         | 30-35       |
| Cr          | Fe           | Cu           | Ti                   | A1                  | Co          |
| 19-23       | Bal.         | .75<br>max.  | 8-10C<br>.40<br>max. | 4-8C<br>.40<br>max. | .10<br>max. |
| Ni          | Cr           |              |                      |                     |             |
| 30-35       | 19-23        |              |                      |                     |             |

It is also recommended that B-0 Alloy material for these structures should be solution annealed at 2150° F.

**BRIEF DESCRIPTION OF THE DRAWINGS**

For a better understanding of this invention, both as to its organization and as to its method of operation, together with additional objects and advantages thereof, reference is made to the following description taken in connection with the accompanying drawings, in which:

FIG. 1 is a view in longitudinal section of a fuel element in which the alloy according to this invention is included and which is made in the practice of the method of this invention;

FIG. 2 is a view in perspective of a tube-to-tube sheet assembly in which the alloy according to this invention is included and in the making of which the method of the invention is practiced;

FIGS. 3, constitutes a plan view and a view in side elevation of a typical sheet of a tube-to-tube sheet assembly as shown in FIG. 2, prepared for welding, and is included for the purpose of aiding those skilled in the art in practicing this invention and not with any intention of in any way limiting this invention;

FIG. 4 is a photomicrograph (at magnification 500X) of a specimen of the prior art iron-nickel-chromium alloy solution annealed at 2,100° F.;

FIG. 5 is a similar photomicrograph of a specimen of this alloy;

FIG. 6 is an electron micrograph (at magnification 5,900X) of a specimen of this alloy;

FIG. 7 is another electron micrograph (at magnification 12,500X) of a specimen of this alloy;

FIG. 8 is another electron micrograph (at magnification 23,000X) of a specimen of this alloy;

FIG. 9 is an electron diffraction pattern of a precipitate in this alloy;

FIG. 10 is a photomicrograph of a specimen of the weld zone of a fusion weld produced with the alloy from which FIGS. 1 through 9 were derived;

FIG. 10A is an electron micrograph (at magnification 1,500X) of a specimen of this weld zone;

FIG. 11 is an electron micrograph (at magnification 23,000X) of a specimen of plate of another prior art alloy showing precipitate concentrated at grain boundaries;

FIG. 12 is a photomicrograph (at magnification 500X) of a specimen of bar stock of alloy according to this invention (B-0 Alloy);

FIGS. 13, 14 and 15 are electron micrographs (at magnifications 6,000X, 13,600X and 24,000X respectively) of this alloy;

FIGS. 16 and 17 are electron micrographs (at magnifications 6,000X and 13,600X respectively) of a specimen of tubing of the iron-nickel-chromium alloy to which were welded lugs of the bar stock whose micrographs are shown in FIGS. 12 through 15 and the welds were found to be crack-free;

FIG. 18 is a photomicrograph (at magnification 500X) of a specimen of this tubing; and

FIGS. 19 through 27 are photomicrographs (at magnification 50X) of welds produced in joining by TIG welding, with fillers of different compositions, parts of iron-nickel-chromium alloy at least one of which was composed of the alloy according to this invention (B-0 Alloy).

#### DESCRIPTION OF PREFERRED EMBODIMENTS

The alloy of this invention is used in, and the method is practiced in the making of, fuel elements 51 as shown in FIG. 1. An element 51 includes fuel pellets 53 contained in cladding. The cladding includes a shell 55 of B-0 Alloy which is sealed by plugs 57 of B-0 Alloy by circumferential welds 59. Insulating spacers 61 are interposed between the fuel pellets 53 and the plugs 57.

The fuel pellets 53 generate intense heat which is transferred to a heat exchange fluid (not shown), typically sodium, in which the fuel element 51 is immersed. The cladding typically has a thickness of 0.010 inches to 0.015 inches. The plugs are welded to the shell by fusion welding with a non-consumable electrode in a shield or atmosphere of inert gas (TIG welding) which may be argon or helium. Welding-grade pure gas is used (99.999 percent) purity. Typically, the process taught in U.S. Pat. No. 3,183,066 Lessman et al. dated May 11, 1963 and in application Ser. No. 603,389 filed Dec. 20, 1966 to Donald R. McClintock continuation of application Ser. No. 275,884, filed Apr. 26, 1963 now abandoned. To prevent the sodium from penetrating into the element, it is necessary that the material of which the cladding 55-57 is composed shall not be corroded by the sodium at high temperatures and that the welds be crack-free. High tensile strength and ductility are also demanded. Cladding composed of the B-0 Alloy meets these conditions.

FIG. 2 shows a tube-to-tube sheet assembly 71 including sheet 73 and tubes 75 welded pressure-tight into the sheet 73 by circumferential welds 77. The sheet 73 is composed of B-0 Alloy and may also be composed of AISI-304 stainless steel. The tubes 75 are composed of B-0 Alloy. Satisfactory welding is carried out by TIG fusion welding with the shoulder of a trepanned groove (81 FIG. 3) providing the filler material. For this welding, a groove 81 is trepanned around the hole 83 into which a tube 75 is to be sealed. Typical dimensions of a sheet 73 with the hole 83 and groove 81 are presented in FIG. 3.

High temperature corrosion resistant material and crack-free welds are necessary because the tubes 75 carry liquid sodium at a high temperature (1,150° F.) and are typically immersed in highly corrosive steam at a high temperature. The B-0 Alloy meets these conditions and in addition has the necessary high tensile strength and ductility at high temperatures.

At the inception of the work from which this invention arose, attempts were made to produce TIG welds

for fuel element cladding with Incoloy-800 alloy having the following composition to evaluate the weldability of this alloy:

TABLE III

| C     | Mn    | Fe    | S     | Si  | Cu  |
|-------|-------|-------|-------|-----|-----|
| .04   | .87   | 47.78 | 0.007 | .47 | .49 |
| Ni    | Cr    | Al    | Ti    |     |     |
| 30.42 | 19.90 | 0.3   | 0.1   |     |     |

5 The specimens for study were TIG welds on flat-plate specimens without filler. Metallographic examination revealed severe cracking in the weld zone occurring generally at weld puddle grain boundaries (FIG. 10). A distinct segregated phase not identifiable by carbon extraction replication techniques was observed within each grain. It was noted that only one type of precipitate was present in the weld puddle metal, i.e., the dendritic structure,  $Cr_{23}C_6$ , in an early stage of structure formation (FIG. 10A). The Incoloy-800 alloy proved to be crack sensitive.

10 A study was made of the alloy. From photomicrographs (not shown) of sections of tubing of the 800 alloy, it was at once noted that sizable precipitates were present near the inner and outer peripheries of the tubing. These precipitates appeared in original specimens and to a lesser extent in specimens solution-annealed at 2,100° F. The photomicrographs and electron micrographs, FIGS. 4 through 8, were then produced from specimens of the alloy annealed for 15 minutes at 1,800° F. and then for one hour at 2,100° F. The micrographs, FIGS. 4 and 5, showed that carbides and nitrides of titanium were formed and that there were other massive carbides which seemed to be coextensive with the grain boundaries. FIGS. 6, 7, and 8 are extraction replications, FIG. 6 shows TiC and TiN and a chromium carbide precipitate. FIG. 7 shows the precipitate in detail and FIG. 8 shows that it is dendritic. The dendritic precipitate was identified from its electron diffraction pattern as  $Cr_{23}C_6$ .

15 It was concluded that the crack sensitivity was caused by the chromium carbide and could be eliminated by suppressing the formation of this carbide. This object is accomplished according to this invention by providing an alloy with adequate titanium and/or aluminum to suppress the formation of chromium carbide.

#### EXAMPLE A

This example covers a comparison of Incoloy-800 and B-0 Alloy. The following structures were used in 20 this comparison:

1. one-fourth inch thick plate of Incoloy-800 alloy.
2. five-eighths diameter bar stock of B-0 Alloy.
3. 0.010 inch thick, 0.400 inch outside diameter tubing.

25 The compositions of items 1 and 2 are given in Table IV:

TABLE IV

| Material                                   | C     | Mn    | S    | Si  | Cr    |
|--------------------------------------------|-------|-------|------|-----|-------|
| 60 $\frac{1}{4}$ " dia. bar<br>B-0 Alloy   | .06   | .91   | .010 | .46 | 20.54 |
| $\frac{1}{4}$ " thick plate<br>Incoloy-800 | .04   | .87   | .007 | .47 | 19.90 |
| Material                                   | Ni    | Fe    | Cu   | Al  | Ti    |
| 65 $\frac{1}{4}$ " dia. bar<br>B-0 Alloy   | 30.10 | 46.47 | .57  | .40 | .48   |
| $\frac{1}{4}$ " thick plate<br>Incoloy-800 | 30.42 | 47.41 | .49  | .30 | .10   |

TABLE V

|                  | C   | Mn   | S    | Si  | Ni    | Cr    | Co   | Ti   | Al    | Cu  | Fe    |
|------------------|-----|------|------|-----|-------|-------|------|------|-------|-----|-------|
| Incoloy-800..... | .05 | 1.06 | .007 | .52 | 30.89 | 21.32 | .10  | .034 | .025  | .45 | 45.09 |
| B-0 alloy.....   | .05 | .65  | .012 | .31 | 31.86 | 20.10 | .178 | .420 | ..... | .21 | 46.79 |

Item 3 was not analyzed chemically. Parts of item 1 were fusion butt welded by TIG welding. End plugs were machined from item 2 and fusion welded by TIG welding to the 0.010 inch wall tubing, item 3. Each weld was sectioned and examined metalographically in 0.003 inch increments. Cracks were observed in the welds of item 1; no cracks were observed in the seal welds of items 2 and 3.

The crack sensitivity of item 1 and the freedom from crack sensitivity of the welds of item 2 and item 3 were

10 The alloys of Table V were evaluated for weldability by producing welds and examining them. The Incoloy-800 alloy was found to be crack sensitive, the B-0 Alloy crack free.

#### EXAMPLE C

15 The weldability of parts of B-0 Alloy to parts of other iron-nickel-chromium alloys with different fillers was evaluated. For this purpose, 2 inch wide  $\times$   $\frac{1}{4}$  inch thick bars were produced of alloys having the compositions shown in Table VI:

TABLE VI

|                | C    | Mn   | Fe    | S    | Si  | Cu  | Ni    | Cr    | Al    | Ti   | P     | Mo    |
|----------------|------|------|-------|------|-----|-----|-------|-------|-------|------|-------|-------|
| B-0 alloy..... | .040 | 1.01 | 46.38 | .009 | .23 | .46 | 30.98 | 20.10 | .44   | .33  | .013  | ..... |
| 304 SS.....    | .058 | 1.52 | Bal.  | .014 | .60 | .29 | 9.50  | 18.65 | ..... | .025 | ..... |       |
| 316 SS.....    | .045 | 1.70 | Bal.  | .016 | .55 | .31 | 12.30 | 17.40 | ..... | .026 | 2.35  |       |

found to be attributable to the presence of  $\text{Cr}_{23}\text{C}_6$  in item 1 and its substantial absence in items 2 and 3 by

Welds were made by TIG welding with the filler materials (wires) shown in Table VII:

TABLE VII

|                  | C    | Mn   | P     | S    | Si  | Cr    | Ni    | Fe   | Cu    | Ti    | Al    | Mo    |
|------------------|------|------|-------|------|-----|-------|-------|------|-------|-------|-------|-------|
| NI 82.....       | .036 | 3.05 | ..... | .005 | .25 | 20.12 | 72.84 | .55  | .06   | .57   | 0.12  | ..... |
| ER 330 SS.....   | .200 | 1.90 | .014  | .012 | .41 | 15.62 | 34.00 | Bal. | ..... | ..... | 3-4.5 |       |
| Incoloy 138..... | .250 | 2.00 | ..... | .025 | .75 | 28.00 | 38.00 | Bal. | .05   | ..... | ..... |       |

metallographic observation. FIG. 11 shows two types of precipitates concentrated at the grain boundaries of specimens of item 1:  $\text{Ti}(\text{C},\text{N})$  and  $\text{Cr}_{23}\text{C}_6$ . In addition, FIG. 11 shows  $\text{Ti}(\text{C},\text{N})$  dispersed throughout the matrix.

FIGS. 12 through 15 show  $\text{Ti}(\text{C},\text{N})$  precipitate dispersed throughout the matrix of specimens of item 2, but substantially no  $\text{Cr}_{23}\text{C}_6$ .  $\text{Ti}(\text{C},\text{N})$  is the major precipitate present in item 3 although there are indications of the  $\text{Cr}_{23}\text{C}_6$  type in an early stage of formation. The  $\text{Ti}(\text{C},\text{N})$  appears larger than in item 2 and is dispersed throughout the matrix.

#### EXAMPLE B

This example covers another comparison of Incoloy-800 and B-0 Alloy. The compositions of the alloys are shown in the following Table V:

35 The weld joints were butt welds made by fusion TIG welding the root pass across the 2 inch face and then filling the joint with filler wire.

40 Two sections of each weld were mounted for metallographic evaluation. All welds were sound and crack free. Typical photomicrographs are shown in FIGS. 19 through 27.

45 Additional samples of each material combination and filler wire were tested by bending 160° around a 1.0 inch diameter mandrel. Results of the bend test are summarized in the following Table VIII:

TABLE VIII

| Material Combination     | Filler Wire | Location of Bend At weld  | Remarks   |
|--------------------------|-------------|---------------------------|-----------|
| B-0 alloy to Inco 138-Ni | .....       | .....                     | No cracks |
| B-0 alloy to 82-330      | 82-330      | .....                     | .....     |
| B-0 alloy to Inco 138-Ni | .....       | On B-0 alloy side of weld | .....     |
| 304 SS 82-330            | 82-330      | .....                     | .....     |
| B-0 alloy to Inco 138-Ni | .....       | On B-0 alloy side of weld | .....     |
| 316 SS 82-330            | 82-330      | .....                     | No cracks |

55 Elevated temperature tensile properties (1,150° F.) of welded specimens are given in the following Table IX:

TABLE IX.—ELEVATED TEMPERATURE TENSILE PROPERTIES 1150° F.

| Material         | Area (sq. in.) | Yield (p.s.i.) | Ultimate (p.s.i.) | Total elong. (percent) | Uniform elong. (percent) | Failure site |
|------------------|----------------|----------------|-------------------|------------------------|--------------------------|--------------|
| B-0-304-82.....  | .09193         | 15,500         | 51,400            | 40.2                   | 36.4                     | 304          |
| B-0-304-82.....  | .09128         | 15,600         | 47,400            | 22.4                   | 21.7                     | 304          |
| B-0-304-138..... | .09232         | 14,600         | 48,750            | 31.6                   | 31.0                     | 304          |
| B-0-304-138..... | .09226         | 21,650         | 43,100            | 38.5                   | 31.2                     | 304          |
| B-0-304-330..... | .09225         | 14,100         | 47,150            | 22.9                   | 22.4                     | Weld         |
| B-0-304-330..... | .09213         | 14,400         | 41,450            | 16.7                   | 16.0                     | 304          |
| B-0-316-82.....  | .09184         | 14,150         | 43,550            | 19.0                   | 18.4                     | Weld         |
| B-0-316-82.....  | .09198         | 14,150         | 53,250            | 25.2                   | 23.9                     | Weld         |
| B-0-316-138..... | .09157         | .....          | 26,500            | 6.8                    | .....                    | Weld         |

Table IX—Continued  
ELEVATED TEMPERATURE TENSILE PROPERTIES 1150° F.

| Material         | Area<br>(sq. in.) | Yield<br>(p.s.i.) | Ultimate<br>(p.s.i.) | Total<br>elong.<br>(percent) | Uniform<br>elong.<br>(percent) | Failure<br>site |
|------------------|-------------------|-------------------|----------------------|------------------------------|--------------------------------|-----------------|
| B-0-316-138..... | .8994             | 15,550            | 56,150               | 25.0                         | 24.7                           | Weld            |
| B-0-316-330..... | .08865            | 15,250            | 48,500               | 26.7                         | 20.1                           | B-0             |
| B-0-316-330..... | .09236            | 14,900            | 47,350               | 18.1                         | 17.3                           | Weld            |
| B-0-800-82.....  | .09204            | 13,900            | 26,200               | 14.5                         | 11.2                           | Weld            |
| B-0-800-82.....  | .09138            | 13,150            | 42,950               | 22.8                         | 22.0                           | Weld            |
| B-0-800-138..... | .09161            | 13,753            | 35,500               | 14.2                         | 13.3                           | Weld            |
| B-0-800-138..... | .09178            | 14,150            | 45,200               | 36.8                         | 36.0                           | Weld            |
| B-0-800-330..... | .09210            | 14,000            | 48,300               | 38.4                         | 30.9                           | Weld            |
| B-0-800-330..... | .09186            | 14,150            | 54,150               | 42.0                         | 37.4                           | B-0             |

These were made with a typical specimen in the form 15  
an I the ends of which flare into the web.

#### EXAMPLE D

A tube-to-tube sheet mock-up as shown in FIG. 2 was 20  
fabricated to illustrate weldability of B-0 Alloy. The  
mock-up consisted of two tube sheets 73, 1 inch thick  
respectively of 304 stainless steel and B-0 Alloy. Tubes  
75 of B-0 Alloy but with high-carbon content were  
welded to the tube sheets 73 by fusion welding and with  
filler wire addition.

Chemical compositions of tube sheet alloys and of  
the tube alloys are given in Table X:

TABLE X

|             | C     | Mn    | Fe    | S     | Si    | Cu   | 30 |
|-------------|-------|-------|-------|-------|-------|------|----|
| B-0 Alloy   |       |       |       |       |       |      |    |
| Tube Sheet  | 0.040 | 1.02  | 44.94 | .008  | 0.28  | 0.47 |    |
| High-Carbon |       |       |       |       |       |      |    |
| B-0 Alloy   |       |       |       |       |       |      |    |
| Tube        | 0.070 | 1.07  | 45.74 | .007  | 0.37  | 0.27 | 20 |
| 304 Tube    |       |       |       |       |       |      |    |
| Sheet       | 0.044 | 1.61  | 69.90 | .012  | 0.51  | 0.27 | 30 |
|             |       |       |       |       |       |      |    |
|             | Ni    | Cr    | Al    | Ti    | P     |      |    |
| B-0 Alloy   |       |       |       |       |       |      |    |
| Tube Sheet  | 31.92 | 20.20 | 0.59  | 0.51  | 0.013 |      |    |
| High-Carbon |       |       |       |       |       |      |    |
| B-0 Alloy   |       |       |       |       |       |      |    |
| Tube        | 30.25 | 21.21 | 0.48  | 0.51  |       |      | 25 |
| 304 Tube    |       |       |       |       |       |      |    |
| Sheet       | 9.41  | 18.22 |       | 0.022 |       |      | 35 |

Welds were performed of the high-carbon B-0 Alloy  
tubes to the tube sheets of B-0 Alloy and of 304 stain- 45  
less steel in accordance to the following schedule:

- 1-TIG fusion tre-pan weld trepanning as shown in  
FIG. 3 — No filler addition
- 2-TIG fusion fillet welds — No filler addition

c. 2-TIG fillet welds — Ni 82 filler wire  
d. 2-TIG fillet welds — 330 filler wire The following  
results were observed by visual examination:  
1. No cracks seen in tre-pan welds of high-carbon B-0  
Alloy tubes to 304 stainless steel and B-0 Alloy  
tube sheets. 2. Microcracks were present in TIG  
fusion fillet welds. 3. Microcracks were present in  
TIG fillet welds with Ni 82 and 330 filler wire addi-  
tions.

It is indicated that the microcracking resulted from  
the high carbon content (0.07) of the high-carbon B-0  
Alloy. In addition, the fillet-type weld with or without  
filler wire imposes high stresses on the weld puddle during  
cooling, resulting in microcracking and the welding of  
tubes into tube-sheet without trepanning is notori-  
ously difficult.

While preferred embodiments of this invention have  
been disclosed herein, many modifications thereof are  
possible. This invention then is not to be restricted ex-  
cept insofar as is necessitated by the spirit of the prior  
art.

I claim as my invention :

- An iron-nickel-chromium alloy having substan-  
tially the following composition in weight percent:

| C   | Mn  | S    | Si  | Cr    | Ni    | Fe    | Cu  | Al  | Ti  |
|-----|-----|------|-----|-------|-------|-------|-----|-----|-----|
| .06 | .91 | .010 | .46 | 20.54 | 30.10 | 46.47 | .57 | .40 | .48 |

for producing welded structures formed by arc welding,  
wherein the welds are substantially free of cracks,  
the said alloy being characterized by including suffi-  
cient content of said carbon affinity elements to sub-  
stantially reduce the formation of chromium carbide.

\* \* \* \* \*